# EUROPEAN PATENT APPLICATION

(11) **EP 2 050 526 A1**
(43) Date of publication of application: **22.04.2009**
(21) Application number: 07020457.3
(22) Date of filing: 18.10.2007
(51) Int. Cl.: B22F 3/10, C21D 1/76, C22F 1/02

(54) **Atmosphere for sintering, annealing or hardening comprising silane or borane**

(71) Applicant: Linde Aktiengesellschaft, 80807 München (DE)
(72) Inventor: Öhrling, Johan, 12638 Hägersten (SE)
(74) Representative: Gellner, Bernd

(57) **Abstract**

The invention relates to a method for sintering or annealing of metal components in a furnace atmosphere comprising nitrogen, hydrogen, argon or any mixture of these gases, each with an addition of a gaseous hydride such as silane or borane.

## Description

The invention relates to a method for sintering or annealing of metal components in a furnace atmosphere comprising one or more of the gases nitrogen, hydrogen and argon.

Metal sintering is defined as the thermal treatment of a metal powder or a mixture of metal powders at an enhanced temperature for the purpose of increasing its strength by bonding together of the particles. During sintering atomic diffusion takes place and the powder particles are welded together. The sintering operation has normally to be carried out under a protective atmosphere in order to prevent oxidation and to promote the reduction of surface oxides.

Annealing is a heat treatment that alters the micro structure of a metal causing changes in properties such as strength and hardness.

The controlled atmosphere for sintering may be produced by blending pure nitrogen with pure hydrogen. In practice such atmospheres contain about 90% nitrogen and 10% hydrogen, sometimes with small additions of CH₄.

The controlled atmosphere for annealing may be produced by blending pure nitrogen with pure hydrogen. In practice such atmospheres contain about 95% nitrogen and 5% hydrogen for carbon steel and 75 to 100% hydrogen and rest nitrogen for stainless steel.

Beside the described synthetic nitrogen-hydrogen atmosphere, today the sintering atmosphere is often produced by the reaction of a hydrocarbon gas with a limited amount of air. Since this reaction is endo-thermic, external heat has to be supplied, and the resulting atmosphere is called endogas. That endogas may contain up to 40% of hydrogen, some carbon monoxide and carbon dioxide with the remainder being nitrogen.

In the production of metal components of good quality, consistency and properties it is advantageous to use an atmosphere with a very low oxygen content and a low dew point. For high quality applications a controlled atmosphere with an water content or oxygen content below 10 ppm or even less is required. However, the production of such pure atmospheres is elaborate and expensive.

Thus it is an object of the invention to develop an improved furnace atmosphere for sintering, hardening or annealing of metal components.

This object is achieved by a method for heat treating of metal components in a furnace atmosphere comprising one or more of the gases nitrogen, hydrogen and argon, which is characterized in that said furnace atmosphere comprises a gaseous hydride.

Gaseous hydrides such as silane are known to have a very high reactivity with oxygen containing substances or compounds. For example, at room temperature silane or mono silane undergoes a spontaneous reaction with oxygen as well as with air:

SiH₄ + O₂ ----> SiO₂ + 2 H₂

SiH₄ + 2 H₂O ----> SiO₂ + 4 H₂

By the inventive addition of a gaseous hydride to the furnace atmosphere any oxygen or water vapour in the atmosphere reacts with the gaseous hydride. Thus it is possible to produce atmospheres with an extremely low dew point and low partial pressure of oxygen.

The invention relates to the heat treatment of metal components. The term "heat treatment" shall mean a method alter the physical or chemical properties of the metal component, in particular sintering, annealing, hardening, tempering and quenching. The term "heat treatment" applies only to processes where the heating and cooling are done for the specific purpose of altering properties intentionally.

Preferably silanes or boranes are added to the furnace atmosphere. Silanes are chemical compounds of silicon and hydrogen. The lowest silanes, mono silane with the chemical formula SiH₄ and di silane with the chemical formula Si₂H₆, are gaseous and thus are particularly suitable for the invention.

Boranes are chemical compounds of boron and hydrogen. The two smallest members of the borane group are mono borane or simply borane BH₃ and di borane B₂H₆. All these compounds are known to be very reactive with oxygen and air. Thus, these boranes are also preferably used for reducing the oxygen content in the furnace atmosphere.

The amount of the gaseous and reactive hydride which is added to the furnace atmosphere is preferably between 0.00001 % and 2 %, most preferably between 0.001 % to 0,05%. The amount of hydride is determined based on one or more of the following factors:
- quality of the atmosphere prior to the addition of the hydride,
- required level of oxygen and water in the furnace atmosphere,
- temperature within the furnace,
- amount of air ingress into the furnace.

It is advantageous to set the furnace temperature between 300 and 1500 °C for the inventive sintering or annealing application.

According to the invention it is possible to extremely decrease the oxygen and moisture level in the furnace atmosphere. Thus, it is possible to subject metals to a heat treatment process which could not have been treated in this way before. In particular, the invention allows to sinter or anneal metal components, in particular steel, without getting the material oxidized or/and discouloured.

In general, the invention is useful for the heat treatment of all kind of metals. Examples for preferred metals and metal powders to be used with the inventive method are iron, low alloyed steel, austenitic, ferritic and duplex stainless steel, copper and copper alloys, nickel and nickel alloys.

In the prior art the controlled atmosphere for annealing may be produced by blending pure nitrogen with pure hydrogen. In practice such atmospheres contain about 95% nitrogen and 5% hydrogen for carbon steel and 75 to 100% hydrogen and rest nitrogen for stainless steel.

According to a preferred embodiment of the invention a little amount of silane is added to the furnace atmosphere. In this case the hydrogen content of the atmosphere can be essentially reduced. For heat treating carbon steel the atmosphere will preferably contain pure nitrogen with addition of silane, and for the heat treatment of stainless steel the furnace atmosphere will consist of about 5-10% hydrogen, a small amount of silane and the remainder being nitrogen.

The inventive furnace atmosphere is either plain nitrogen, plain hydrogen, plain argon or a mixture of these gases blended with a gaseous hydride. Preferred furnace atmospheres are
- plain nitrogen,
- a mixture of an inert gas and hydrogen,
- a mixture of nitrogen and hydrogen,
- a mixture of argon and hydrogen,
- a mixture of nitrogen, argon and hydrogen,
wherein to each of the above atmospheres a gaseous hydride, especially silane, is added.

The mixture of nitrogen and hydrogen or the mixture of argon and hydrogen are preferably produced by blending pure nitrogen with hydrogen or pure argon with hydrogen, respectively. Nitrogen/hydrogen mixtures may also be produced by endothermic generators or ammonia dissociation.

The invention is particularly advantageous for the production of a controlled atmosphere in industrial furnaces, for example in a continuous furnace for heat treatment of metals. In such furnaces there is always some leak air entering the furnace increasing the oxygen and water vapour content of the furnace atmosphere. By the inventive addition of a gaseous reactive hydride any ingress of air and moisture reacts with the hydride so that within the furnace a high quality atmosphere is permanently guaranteed.

The inventive method is not only useful to decrease the oxygen and water vapour content in a furnace atmosphere but can also be used as a reducing agent to react with other impurities in the atmosphere, for example organic compounds.

Annealing of steel in the inventive atmosphere is a good alternative to pickling of stainless steel. By using the inventive atmosphere the amount of oxides on the surface of the steel can be essentially reduced.

Another preferred application of the invention is sintering of powder containing easily oxidised elements like chromium, manganese and silicon.

## Claims

1. Method for heat treatment of metal components in a furnace atmosphere comprising one or more of the gases nitrogen, hydrogen and argon, **characterized in that** said furnace atmosphere comprises a gaseous hydride.

2. Method according to claim 1 **characterized in that** said furnace atmosphere comprises silane or borane.

3. Method according to any of claims 1 or 2 **characterized in that** the concentration of said gaseous hydride in said furnace atmosphere is between 0.00001 % and 2 %, preferably between 0.001% to 0,05%.

4. Method according to any of claims 1 to 3 **characterized in that** said sintering or annealing is carried out at a temperature between 300 and 1500 °C.

5. Method according to any of claims 1 to 4 **characterized in that** said sintering or annealing is carried out in an industrial furnace.

6. Method according to any of claims 1 to 5 **characterized in that** said furnace atmosphere essentially consists of
- nitrogen and said gaseous hydride or of
- argon, hydrogen and said gaseous hydride or of
- an inert gas and hydrogen and said gaseous hydride.
